

106-98xx.

S. W. FLESHEIM.

METHOD OF BONDING CONCRETE.

APPLICATION FILED JUNE 19, 1911.

1,012,832.

Patented Dec. 26, 1911.

72-106



WITNESSES:

Bernard B. Went.  
Edith Smith

INVENTOR,  
Sylvester W. Flesheim  
BY Hull & Smith  
ATTYS.

# UNITED STATES PATENT OFFICE.

SYLVESTER W. FLESHEIM, OF CLEVELAND, OHIO, ASSIGNOR TO THE MASTER BUILDERS COMPANY, OF CLEVELAND, OHIO, A CORPORATION OF OHIO.

## METHOD OF BONDING CONCRETE.

1,012,832.

Specification of Letters Patent. Patented Dec. 26, 1911.

Application filed June 19, 1911. Serial No. 634,028.

**REISSUED**

*To all whom it may concern.*

Be it known that I, SYLVESTER W. FLESHEIM, a citizen of the United States, residing at Cleveland, in the county of Cuyahoga and State of Ohio, have invented a certain new and useful Improvement in Methods of Bonding Concrete, of which the following is a full, clear, and exact description, reference being had to the accompanying drawings.

This invention relates to cement or concrete structures and has for its object the production of a process whereby a new cement or concrete structure can be economically and permanently affixed to a previously existent structure or mass of the same material.

It is frequently necessary in building or altering operations to build a new cement wall or facing upon a mass of concrete which has already hardened and perhaps been worn by traffic or eroded by the weather. An instance of this condition is the laying of a new concrete flooring upon a concrete floor which has already become worn or marred. Heretofore it has always been necessary to break or chisel away a considerable amount of the old structure, both for the purpose of producing a rough and uneven surface upon which the fresh concrete can become bonded, and to render the thickness of such new coating sufficiently great to prevent its peeling away by reason of its contraction, or its being broken up by blows and shocks.

The object of this invention is the production of a process of treating the surface of an old structure so that newly laid cement will be firmly and permanently affixed thereto, even though the thickness of the new coating be comparatively slight, thus markedly cheapening and facilitating the operation of resurfacing or adding to the previous structure.

The invention consists in the process hereinafter fully described and pointed out in the claims.

I have discovered that when a plastic mass containing finely divided corrodible metal particles is spread upon the surface of the already existing concrete structure, the portion of that plastic mass adjacent to the surface of the old structure will penetrate into the pores thereof and will thereafter become oxidized and swell up so as

to become firmly interlocked therewith, and that if the new coating or the new structure be laid upon this plastic coating before the same has thoroughly set, it will in its turn become firmly anchored thereto in the same manner, so that when the whole mass becomes dried and hardened it will be permanently fixed in place. In preparing this plastic mass I preferably employ a mixture of finely divided metallic iron and pulverized cement and dry sal-ammoniac substantially in the following proportions.

|              |        |    |
|--------------|--------|----|
| Iron         | 49-47% | 70 |
| Cement       | 49-47% |    |
| Sal-ammoniac | 2-6%   |    |
| 100-100      |        |    |

When I desire to employ the same I mix it with water to the consistency of a rather thin dough which can be spread with a trowel to a thickness of from one-sixteenth inch upward and I preferably work the same thoroughly into contact with all parts of the old structure. The new coating is then applied in the usual way either by pouring or by troweling as may be most convenient, care being taken to apply the same before the first or "slush" coating has had a chance to set. This slush coating is usually made rather thin in order to save expense, as a thin coating will anchor the new cement as thoroughly as a thicker coating, since it is the surface action only which is important.

The proportions above named are not invariable but may be widely varied without departing from the scope of my invention or losing the benefits of my process. In many instances it will be found possible to employ a slush coating containing a smaller amount of iron, especially where the wear expected is not heavy, and, conversely, a much richer coating can be employed if desired. In fact the cement can be entirely dispensed with in many instances although I prefer to employ the same in order to thicken the mixture and hold the iron particles in suspension during the time of their application as well as to cheapen the process. The sal-ammoniac is employed solely for the purpose of expediting the oxidation of the iron particles, although other oxidizing agents may obviously be employed, or in fact entirely omitted although with a

corresponding increase in the time required to allow the coating to set. Sand can also be added to the mixture in order to dilute and cheapen the same.

5 In case I am resurfacing a floor, I prefer to mix the cement coating also with a small percentage of the same finely divided particles, with or without the use of sal-ammoniac, inasmuch as this expedient produces a concrete of very great hardness and wearing qualities, although the operation of the slush coating is exactly the same whether or not the cement coating be thus treated. It is preferable, however, to employ a small 10 admixture of the iron particles in the second or cement coating in all cases in which this coating is to be of small thickness, whether it is to be used as a floor or not, since the expansion of the iron particles due to their 15 oxidation will be found to compensate in a large measure the shrinkage of the cement due to its drying and hardening, and so diminish its tendency to curl up and peel away from the surface to which it is applied.

20 25 In the drawing accompanying and forming a part of this application I have illustrated the application of my new method of bonding cement under several different conditions of use. This drawing illustrates a portion of a concrete floor and of a wall built up of concrete blocks, the blocks being secured together with a mortar made according to my invention and both the floor and wall being covered with a facing or surface layer of cementitious material bonded thereto in accordance with my invention. The blocks are shown at 1, the mortar between them at 2, the slush coat of bonding material at 3, the original concrete floor at 40 4, the floor topping at 5, and the wall facing at 6. The mortar shown at 2 is composed of exactly the same ingredients as the slush coat above described, but is preferably considerably poorer in iron and richer in cement, in order that its body and consistency may be increased. The effect of the iron particles in penetrating into the pores of the concrete blocks is illustrated at 2<sup>a</sup>.

The original floor 4 is supposed to have 50 been laid after the building of the side wall according to the usual practice, and to have been bonded thereto in accordance with my invention by means of a slush coat indicated in cross section at 3<sup>a</sup>, thus causing the firm 55 adherence of these parts and preventing such a breaking away as would permit the entrance of water or vermin therein. The method of spreading the slush coat 3 and of applying the topping 5 and facing 6 will 60 be apparent to any one skilled in the art from the preceding description and further elucidation is believed to be unnecessary.

While I have specified iron as the material which I prefer to use it is obvious that other 65 corrodible metals may be employed in case

they be such as will expand upon corrosion, but the cheapness and accessibility of iron renders it particularly desirable. Other corrodible agents than sal-ammoniac may also obviously be employed and may be added either in the dry state before mixing with water or may be added to the water and employed in solution.

70 While I have described my process as employed with cement structures it is obvious that it may be employed with structures of any porous material such as brick or stone with satisfactory results. It will also be found that if a mortar of cement mixed with finely divided iron particles be employed 75 between already formed porous structures such as concrete blocks, the adhesion of the same will be much improved by reason of the penetrating and interlocking qualities of the iron particles. While I have necessarily described my invention in detail I do not, therefore, propose to be limited to such details except as the same may be positively included in the claims hereto annexed or may be rendered necessary by the prior state 80 of the art.

85 What I claim as new and desire to secure by Letters Patent of the United States is:—

1. The process of bonding a new cement structure to an already existent porous structure which consists in applying to the surface of the latter structure a coating of cement containing finely comminuted corrodible metallic particles and applying to the surface of such coating in advance of its 90 hardening, a new cement structure whereby said metallic particles may penetrate into the pores of both said structures and become firmly interlocked therewith.

95 100 110 105 2. The process of bonding together two porous cementitious structures which consists in interposing therebetween a plastic mass containing finely divided corrodible metallic particles whereby said metallic particles may penetrate into the pores of said structures and become interlocked therewith upon oxidation so as to bind the two firmly together.

115 120 125 130 3. The process of bonding a new cement structure to an already existing cement structure which consists in applying to the latter structure a plastic coating containing cement and finely divided corrodible metallic particles and a corrodible agent, and applying the new cement structure to the surface of said first coating before the hardening thereof whereby the metallic particles will penetrate the pores of both structures and become firmly interlocked therewith.

4. The process of resurfacing an already existing cement structure which consists in applying to the surface of such structure a plastic coating containing finely divided corrodible metallic particles, and thereafter applying to said coating in advance of the

hardening thereof a surface of cement mixed with finely divided iron.

5. The process of resurfacing an already existing cement structure which consists in applying to the surface of such structure a plastic coating consisting substantially of cement fifty parts, finely divided metallic iron fifty parts and sal-ammoniac two parts mixed with water and of applying a surface

of cement mixed with finely divided iron to 10 said coating in advance of the hardening thereof.

In testimony whereof, I hereunto affix my signature in the presence of two witnesses.

S. W. FLESHEIM.

Witnesses:

W. E. NEWMAN,

A. D. HICKEY.

Copies of this patent may be obtained for five cents each, by addressing the "Commissioner of Patents, Washington, D. C."